# EUROPEAN PATENT SPECIFICATION

(11) **EP 3 110 995 B1**
(45) Date of publication and mention of the grant of the patent: **17.10.2018**
(21) Application number: 15709588.6
(22) Date of filing: 26.02.2015
(51) Int. Cl.: D04H 1/425, D04H 1/4274, E04B 1/74, E04B 2/00

(54) **NONWOVEN PANEL FORMED OF END-OF-LIFE INGREDIENTS AND METHOD OF CONSTRUCTION THEREOF**
AUS ALTBESTANDTEILEN GEFORMTE VLIESTAFEL UND VERFAHREN ZUR KONSTRUKTION DAVON
PANNEAU NON TISSÉ FORMÉ D'INGRÉDIENTS DE FIN DE VIE, ET SON PROCÉDÉ DE CONSTRUCTION

(30) Priority: 26.02.2014 US 201461944851 P
(43) Date of publication of application: 04.01.2017
(73) Proprietor: Federal-Mogul Powertrain LLC, Southfield, MI 48034 (US)
(72) Inventor: LAURENT, Benoit, F-60350 Trosly Breuil (FR); MEHBUBANI, Ritesh, Royersford, PA 19468 (US); BONALDI, Elisa, Bogota (BO); STAUDT, Eric K., Reading, PA 19606 (US)
(74) Representative: HGF Limited
(86) International application number: PCT/US2015/017701
(87) International publication number: WO 2015/130909

(56) References cited:
- WO-A1-2008/086458
- WO-A1-2010/063079
- WO-A2-2010/151627
- US-A1- 2008 121 461
- US-A1- 2011 305 878

## Description

### BACKGROUND OF THE INVENTION

### 1. Technical Field

This invention relates generally to nonwoven materials, and more particularly to nonwoven panels containing recycled ingredients.

### 2. Related Art

Many end-of-life items are presently sent to landfills or incinerated due in large part to their being considered unsuitable for being recycled and/or due to the laborious cost associated with their being recycled, such as sorting and disassembling, for example. Accordingly, landfills are being rapidly filled by these items, which in turn have a detrimental effect on the environment, both from a costly pollution standpoint and from the standpoint of losing any return value on the materials being disposed.

Accordingly, there exists a need for being able to prevent the disposal of end-of-use items, particularly those with high quality material content.

### SUMMARY OF THE INVENTION

In accordance with one aspect of the invention, a nonwoven panel is provided in accordance with the appended claims. The nonwoven panel can be constructed having properties ideally suited for automotive acoustic panels (e.g. headliners, side-door panels, trunk liners, finished interior panels, under carpet padding), or other types of vehicles and their associated acoustic panels.

The nonwoven panel may include a nonwoven mat with a scrim layer laminated to an outer surface of the nonwoven mat.

The seatbelts and airbags from used vehicles and/or professional apparel are gathered and processed via a shredding or tearing operation. The shredded or torn material, referred to hereafter commonly as comminuted material, is sized to provide fibers ranging between about 30-75mm in length, as desired, and having a denier ranging between about 3-10. The comminuted material is blended with low melt fibers, and then the mixture is processed via a nonwoven webbing process, such as in an air laid machine (e.g. Rando air laid machine or an air gravity machine). The air laid machine mixes and forms a randomly oriented fiber web, wherein the web can be further processed in a needling operation and then optionally sent to a heating process (e,g., a heated conveyor oven or batch oven), or it can be sent directly from the air laid process to the heating process, depending on the finish panel structure desired.

In accordance with a further aspect of the invention, the end-of-life material used to form the web can be treated with a compounded mixture including an antimicrobial, a flame retardant, and a binder. The mixture can be applied to the end-of-life material either prior to comminuting the material, after comminuting the material and prior to forming the air laid web, or as a coating on an exposed side of the web after forming web.

In accordance with a further aspect of the invention, the compounded mixture of antimicrobial, flame retardant and binder can be provided having between about 1-4% dry pickup weight.

In accordance with a further aspect of the invention, the nonwoven mat can include between about 50-70 wt% seatbelt fibers.

In accordance with a further aspect of the invention, the nonwoven mat can include between about 30-50 wt% airbag fibers.

In accordance with a further aspect of the invention, the nonwoven mat can include between about 0-50 wt% professional garment fibers.

In accordance with a further aspect of the invention, the nonwoven mat can include between about 15-25 wt% low melt fibers.

In accordance with a further aspect of the invention, the nonwoven web can have a weight ranging between about 200-1000gsm.

In accordance with a further aspect of the invention, the scrim layer can have a weight ranging between about 25-200gsm.

In accordance with a further aspect of the invention, a method of constructing an acoustic, nonwoven panel is provided in accordance with the appended claims.

In accordance with another aspect of the invention, the method can include forming the fibrous mixture containing at least 50 wt% of the first fibers from vehicle seatbelts and at least 30 wt% of the second fibers from vehicle air bags.

In accordance with another aspect of the invention, the method can include forming the fibrous mixture containing between 15-25 wt% of the low melt polymeric material.

In accordance with another aspect of the invention, the method can include forming the mixture containing between 50-70 wt% of the first fibers from vehicle seatbelts.

In accordance with another aspect of the invention, the method can include forming the mixture including between 0-50 wt% of the third fibers from professional garments.

In accordance with another aspect of the invention, the method can include applying a compounded mixture including an antimicrobial, a flame retardant, and a binder to the bonded web.

In accordance with another aspect of the invention, the method can include providing the compounded mixture applied to the web having a dry pickup between 1-4 wt%.

In accordance with another aspect of the invention, the method can include bonding a scrim layer to the bonded web.

In accordance with another aspect of the invention, the method can include providing the scrim layer having a weight between 25-200gsm.

In accordance with another aspect of the invention, the method can include first coating the bonded web with the compounded mixture and then bonding the scrim layer to a single side of the bonded web.

In accordance with another aspect of the invention, the method can include performing the bonding in a needling operation.

In accordance with another aspect of the invention, the method can include performing the bonding in a thermal treatment process.

### BRIEF DESCRIPTION OF THE DRAWINGS

These and other aspects, features and advantages of the present invention will become more readily appreciated when considered in connection with the following detailed description of presently preferred embodiments and best mode, appended claims and accompanying drawings, in which:
Figure 1 is a process flow diagram of a process used to construct an acoustic, nonwoven panel from end-of-life material in accordance with one aspect of the invention;
Figure 2 is perspective view of a vehicle containing acoustic, nonwoven panels construction in accordance with one aspect of the invention; and
Figure 3 is a cross-sectioned side view of an acoustic, nonwoven panel from the vehicle of Figure 2.

### DETAILED DESCRIPTION OF PRESENTLY PREFERRED EMBODIMENTS

Referring in more detail to the drawings, Figure 1 illustrates a process flow used to construct an acoustic, nonwoven panel, referred to hereafter as panel 10 (Figures 2 and 3), from end-of-life textile material 12 in accordance with the invention. The process, as shown, is generally a "closed-loop" process that reclaims and reprocesses parts from used, end-of-life parts of vehicles, such as trains and/or automotive vehicles, and in particular, from parts including high quality fibrous end-of-life textile materials, such as of nylon and polyester, including end-of life seatbelts and air bags, and/or from used, end-of-life professional apparel (e.g. imaging apparel). Accordingly, the end-of-life textile material 12 used to construct the panel 10 includes at least one of first fibers 14 from end-of-life vehicle seatbelts, second fibers 16 from end-of-life vehicle airbags and third fibers 18 from end-of-life professional garments. The ability to construct the panel 10, including the reclaimed end-of-life textile material 12, avoids having to send the reclaimed end-of-life material to a landfill or incinerator, thereby negating a negative impact on the environment, while further providing the ability to repurpose the high quality fibrous material from the reclaimed materials 12.

The end-of-life textile parts, namely seatbelts and airbags from used vehicles, and/or professional apparel are gathered and can be bulked together, if desired, and then the gathered materials are processed via a shredding or tearing operation. Of course, the separate types of end-of-life parts can be processed separately, and then mixed afterward, if desired, to allow optimal control of the percent-by-weight (wt%) of the different types of fibers in the resulting mixture. The shredded or torn material, referred to hereafter commonly as comminuted material, is sized as desired to provide fluffy textile fibers of a length ranging between about 30-75mm, and having a denier ranging between about 3-10, depending on the end type of acoustic panel being made. The comminuted end-of-life material can be blended with other textile fibers, including low melt fibers 20, particularly if not already included in the end-of-life materials, along with additional materials, such as organic fibers including natural fibers of jute, kenaf, sisal and the like, and then the mixture is further processed via a nonwoven webbing process, such as in an air laid machine (e.g. Rando air laid machine or an air gravity machine). The air laid machine mixes and randomly orients the fibers with one another to form the fibrous web 22 (Figure 3). The web 22 can then be processed in a needling operation, if desired, to bond or interlock the fibers with one another. The needled web can then be sent to a thermal treatment process (e.g., a heated conveyor oven, batch oven or heated rollers), wherein the low melt fibers 20 are at least partially melted to further bond the fibers with one another, To facilitate providing the web 22 with the desired finished density, the low melt fibers 20 are preferably provided as bi-component fibers, having a low melt outer sheath material encapsulating a high melt temperature inner core material Known bicomponent fibers suitable for use include, by way of example and without limitation, PE/PET, PE/PP, PET/PET (with an outer sheath of PET having a lower melt temperature than the inner core of PET), Accordingly, the outer sheath is melted to bond the fibers of the fibrous mixture with one another, while the inner core remains unmelted or substantially unmelted, thereby enhancing the loft, lightweight, and acoustically absorbent properties of the finished web 22. In accordance with a further aspect of the invention, rather than needling the web 22, the web 22 of fibrous material can be sent directly from the air laid process to the thermal treatment process, depending on the structure of the finished panel 10 desired.

Additional processes can be performed on the web 22 to attain the properties sought in the finished panel 10, depending on the type of use and environment the resulting panel 10 will be exposed to in use. For example, the panel 10 can be prepared for suitable use not only as an acoustical panel, by also for use as a structural panel, finished surface panel, insulation/heat shield panel, or otherwise. In accordance with a preferred embodiment, the bonded web 22 is sent through a chemical application station, such as a spraying, dipping, brushing, or any other type of coating process, by way of example and without limitation, wherein a chemical compounded mixture is applied to an outer surface of the bonded web 22 to form a coating 24 of the compounded mixture on the web 22. The coating 24 can be formed about the entirety of the web 22, or the coating 24 can be formed on a selected portion of the web 22, such as to an outer surface of the web 22 that will remain generally exposed to the environment during use. Accordingly, with the web 22 having opposite sides 26, 28, the coating 24 can be applied over both sides 26, 28, or applied to cover a single side 26 of the web 22, thereby reducing the content and cost of the coating 24 on the finished panel.

The compounded mixture is applied to the web 22 having between about 4-10 wet pickup wt%, which results in a dry pickup between about 1-4 wt%. The compounded mixture includes an antimicrobial agent, a flame retardant agent, and a binder agent. In accordance with a preferred embodiment, the antimicrobial agent has dry pickup wt% between about 0.01-0.05, the flame retardant agent has a dry pickup wt% between about 0.5-2, and the binder has a dry pickup wt% between about 0.5-2. The antimicrobial agent can be provided as any suitable biocide, including dichloroctylisotliiazolinone-based agents, by way of example and without limitation. The flame retardant agent can also be provided as any suitable flame retardant, including, by way of example and without limitation, ammonium sulphate, phosphorous-based, or bromine-based agents. The binder, by way of example and without limitation, can be provided as a styrene butadiene binder (SBR) or an acrylic binder. In alternative to forming the coating 24 to at least one of the outer surfaces 26, 28 of the bonded web 22, the compounded mixture can be applied to the end-of-life material either prior to comminuting the material, after comminuting the material and prior to forming the air laid web, or to the web prior to bonding the fibers of the web.

During the manufacture of the web 22, the process includes controlling the thickness, preferably between about 10-25min and density, preferably between about 200-1000gsm, of the finished web 22, such as via a belt or roller(s), by way of non-limiting example, within the heating oven used to melt the low melt fibers 20 added to, or pre-existing within the end-of-life material, Further, rather than using an oven to perform the heating, the nonwoven web 22 can be heated and sized (thickness and density) between heated rollers, if desired. In addition, sizing can further be controlled by passing the heated web 22 between cooled rollers after the web exits the heating/bonding process.

The panel 10 is shown as having a scrim layer 30 bonded to one side 28 of the web 22. The scrim layer 30 is preferably provided as a microfiber scrim having lamination of spunbond/meltbond/spunbond (SMS) layers, and has a density ranging between about 25-200gsm. The scrim layer 30 is preferably bonded to the side 28 of the web 22 via a hot melt adhesive. The presence of the scrim layer 30 enhances the overall acoustic performance of the panel 10. It should be recognized that the side 28 having the scrim layer 30 bonded thereto can be void of the coating 24, thereby reducing the material and manufacture cost by saving on the expense of the coating chemical composition.

The content by wt% of the first fibers 14, second fibers 16, third fibers 18 and lower melt fibers 20 can be adjusted, within parameters specified herein, to provide the panel 10 with the performance characteristics sought. In accordance with one aspect of the invention, the web 22 can be formed having between about 50-70 wt% of the first fibers 14 and between about 30-50 wt% of the second fibers and between about 15-25 wt% of the low melt fibers 20. Accordingly, in accordance with one preferred embodiment, the panel 10 can be fabricated having at least 50 wt% of the first fibers 14 and at least 30 wt% of the second fibers 16, In accordance with another embodiment of the invention, the web 22 can be fabricated having between about 0-50 wt% of the third fibers 18 from professional garments. In accordance with yet another embodiment of the invention, the web 22 can be fabricated having between about 50-100 wt% of the first and/or second fibers 14, 16.

It should be recognized that various types of end-use panels 10 can be fabricated in accordance with the invention, wherein the panels 10 can be constructed having different constituent ingredients (types of end-of-life materials 12 with selected coatings 24 and scrim layers 30, as desired) and shapes/contours. While heating the web 22 and bonding the ingredients thereof to one another, the resulting contour and peripheral shape can be provided in a cutting and heat forming/compressing operation, wherein precise contour and peripheral shape and dimensions, including thickness over the entirety of the panel 10, whether constant or of varying thickness, can be readily formed.

Many modifications and variations of the present invention are possible in light of the above teachings. It is, therefore, to be understood that the invention may be practiced otherwise than as specifically described, and that the scope of the invention is defined by any ultimately allowed claims,

## Claims

1. A method of constructing an acoustic, nonwoven panel (10), said method comprising:
forming a fibrous mixture including low melt polymeric material (20) and at least 50 wt% of first fibers (14) of vehicle seatbelts and/or at least 30 wt% second fibers (16) from vehicle airbags;
forming a web (22) from said mixture in a nonwoven webbing process; and
bonding fibers (14, 16, 20) within the web (22) with one another.

2. The method of claim 1 further including forming the fibrous mixture containing at least 50 wt% of the first fibers (14) and at least 30 wt% of the second fibers (16).

3. The method of claim 2 further including forming the fibrous mixture containing between 15-25 wt% of the low melt polymeric material (20).

4. The method of claim 1 further including forming the mixture containing between 50-70 wt% of the first fibers (14).

5. The method of claim 1 further including applying a compounded mixture (24) including an antimicrobial, a flame retardant, and a binder to the bonded web (22).

6. The method of claim 5 further including bonding a scrim layer (30) to the bonded web (22).

7. The method of claim 6 further including providing the scrim layer (30) having a weight between 25-1000gsm.

8. The method of claim 1 further including performing the bonding in at least one of a needling operation and a thermal treatment process.

9. An acoustic nonwoven panel (10) obtained by the method of claim 1, comprising:
a bonded fibrous mixture including low melt polymeric material (20) and at least 50 wt% of first fibers (14) of vehicle seatbelts and/or at least 30 wt% second fibers (16) from vehicle airbags, wherein the fibers (14, 16) range between about 30-75mm in length and have a denier ranging between about 3-10.

10. The acoustic nonwoven panel of claim 9 wherein said bonded fibrous mixture is needle punched.

11. The acoustic nonwoven panel of claim 9 wherein said low melt material (20) is at least partially melted and optionally said low melt material is a bi-component fiber (20).

12. The acoustic nonwoven panel of claim 9 wherein said bonded fibrous mixture contains between 50-70 wt% of said first fibers (14).

13. The acoustic nonwoven panel of claim 12 wherein said bonded fibrous mixture contains at least 30 wt% of said second fibers (16).

14. The acoustic nonwoven panel of claim 9 further including a compounded mixture (24) bonded to said bonded fibrous mixture, said compounded mixture (24) including an antimicrobial, a flame retardant, and a binder.

15. The acoustic nonwoven panel of claim 14 further including a scrim layer (30) bonded to said bonded fibrous mixture.

## Patentansprüche

1. Verfahren zur Konstruktion eines akustischen Vliesfeldes (10), wobei das Verfahren Folgendes umfasst:
Formen eines Fasergemischs, enthaltend niedrigschmelzendes Polymermaterial (20) und mindestens 50 Gew.-% erster Fasern (14) aus Fahrzeugsicherheitsgurten und/oder mindestens 30 Gew.-% zweiter Fasern (16) aus Fahrzeugairbags;
Formen eines Flächengebildes (22) aus dem Gemisch in einem Vliesbildungsprozesses; und Bindefasern (14, 16, 20) in dem Flächengebilde (22) miteinander.

2. Verfahren nach Anspruch 1, ferner enthaltend das Formen des Fasergemischs, enthaltend mindestens 50 Gew.-% der ersten Fasern (14) und mindestens 30 Gew.-% der zweiten Fasern (16).

3. Verfahren nach Anspruch 2, ferner enthaltend das Formen des Fasergemischs, enthaltend zwischen 15-25 Gew.-% des niederschmelzenden Polymermaterials (20).

4. Verfahren nach Anspruch 1, ferner umfassend das Formen des Gemischs, enthaltend zwischen 50-70 Gew.-% der ersten Fasern (14).

5. Verfahren nach Anspruch 1, ferner enthaltend das Auftragen eines zusammengesetzten Gemischs (24), enthaltend ein antimikrobielles, ein flammenhemmendes und ein Bindemittel auf das gebundene Flächengebilde (22).

6. Verfahren nach Anspruch 5, ferner enthaltend das Binden einer Gitterschicht (30) an das gebundene Flächengebilde (22).

7. Verfahren nach Anspruch 6, ferner enthaltend das Bereitstellen einer Gitterschicht (30) mit einem Gewicht von zwischen 25-100 g/qm.

8. Verfahren nach Anspruch 1, ferner enthaltend das Ausführen des Bindens in mindestens einem eines Nadelvorgangs und eines Wärmebehandlungsprozesses.

9. Akustisches Vliesfeld (10), das durch das Verfahren nach Anspruch 1 erhalten wurde, umfassend:
ein gebundenes Fasergemisch, enthaltend niederschmelzendes Polymermaterial (20) und mindestens 50 Gew.-% erster Fasern (14) aus Fahrzeugsicherheitsgurten und/oder mindestens 30 Gew.-% zweiter Fasern (16) aus Fahrzeugairbags, wobei die Fasern (14, 16) in der Länge zwischen etwa 30-75 mm variieren und einen Denier im Bereich von etwa 3-10 aufweisen.

10. Akustisches Vliesfeld nach Anspruch 9, wobei das gebundene Fasergemisch vernadelt wird.

11. Akustisches Vliesfeld nach Anspruch 9, wobei das niederschmelzende Material (20) mindestens teilweise geschmolzen wird und optional wobei das niederschmelzende Material eine Bikomponentenfaser (20) ist.

12. Akustisches Vliesfeld nach Anspruch 9, wobei das gebundene Fasergemisch zwischen 50-70 Gew.-% der ersten Fasern (14) enthält.

13. Akustisches Vliesfeld nach Anspruch 12, wobei das gebundene Fasergemisch mindestens 30 Gew.-% der zweiten Fasern (16) enthält.

14. Akustisches Vliesfeld nach Anspruch 9, ferner enthaltend ein zusammengesetztes Gemisch (24), das mit dem gebundenen Fasergemisch gebunden wird, wobei das zusammengesetzte Gemisch (24) ein antimikrobielles, ein flammenhemmendes und ein Bindemittel enthält.

15. Akustisches Vliesfeld nach Anspruch 14, ferner enthaltend eine Gitterschicht (30), die mit dem gebundenen Fasergemisch gebunden ist.

## Revendications

1. Procédé de construction d'un panneau non-tissé acoustique (10), ledit procédé comprenant :
la formation d'un mélange fibreux incluant un matériau polymérique à point de fusion bas (20) et au moins 50 % massique de premières fibres (14) de ceintures de sécurité de véhicule et/ou au moins 30 % massique de secondes fibres (16) provenant d'airbags de véhicule ;
la formation d'une sangle (22) à partir dudit mélange dans un processus de sangle non-tissée ; et le liage de fibres (14, 16, 20) dans la sangle (22) les unes aux autres.

2. Procédé selon la revendication 1, incluant en outre la formation du mélange fibreux contenant au moins 50 % massique des premières fibres (14) et au moins 30 % massique des secondes fibres (16).

3. Procédé selon la revendication 2, incluant en outre la formation du mélange fibreux contenant entre 15 et 25 % massique du matériau polymérique à point de fusion bas (20).

4. Procédé selon la revendication 1, incluant en outre la formation du mélange contenant entre 50 et 70 % massique des premières fibres (14).

5. Procédé selon la revendication 1, incluant en outre l'application d'un mélange composé (24) incluant un antimicrobien, un retardateur de flamme et un liant sur la sangle liée (22).

6. Procédé selon la revendication 5, incluant en outre le liage d'une couche de canevas (30) à la sangle liée (22).

7. Procédé selon la revendication 6, incluant en outre la fourniture de la couche de canevas (30) ayant une hauteur entre 25 et 1000 gsm.

8. Procédé selon la revendication 1, incluant en outre l'exécution du liage dans au moins l'un d'une opération d'aiguilletage et un processus de traitement thermique.

9. Panneau non-tissé acoustique (10) obtenu par le procédé selon la revendication 1, comprenant :
un mélange fibreux lié incluant un matériau polymérique à point de fusion bas (20) et au moins 50 % massique de premières fibres (14) de ceintures de sécurité de véhicule et/ou au moins 30 % massique de secondes fibres (16) provenant d'airbags de véhicule, dans lequel les fibres (14, 16) ont une longueur comprise entre environ 30 et 75 mm et ont un denier situé entre environ 3 et 10.

10. Panneau non-tissé acoustique selon la revendication 9, dans lequel ledit mélange fibreux lié est aiguilleté.

11. Panneau non-tissé acoustique selon la revendication 9, dans lequel ledit matériau à point de fusion bas (20) est au moins partiellement fondu et en option ledit matériau à point de fusion bas est une fibre bicomposée (20).

12. Panneau non-tissé acoustique selon la revendication 9, dans lequel ledit mélange fibreux lié contient entre 50 à 70 % massique desdites premières fibres (14).

13. Panneau non-tissé acoustique selon la revendication 12, dans lequel ledit mélange fibreux lié contient au moins 30 % massique desdites secondes fibres (16).

14. Panneau non-tissé acoustique selon la revendication 9, incluant en outre un mélange composé (24) lié audit mélange fibreux lié, ledit mélange composé (24) incluant un antimicrobien, un retardateur de flamme et un liant.

15. Panneau non-tissé acoustique selon la revendication 14, incluant en outre une couche de canevas (30) liée audit mélange fibreux lié.
